

# United States Patent Office

3,067,159

Patented Dec. 4, 1962

1

3,067,159

## QUEOUS WATER REPELLENT DISPERSIONS COMPRISING A METHYLENE DIALKYL AMIDE, A METHYLOL CONDENSATE, AND A NON-IONIC SURFACE ACTIVE AGENT

David M. Musser, Fairlawn, N.J., assignor, by mesne assignments, to Chicopee Manufacturing Corporation, New Brunswick, N.J., a corporation of Massachusetts  
No Drawing. Filed Oct. 17, 1957, Ser. No. 690,625

10 Claims. (Cl. 260—29.4)

This invention relates to an improvement in durable water repellent finishes for textile fibers and fabrics.

In the durable water repellent finishes for textile fibers and fabrics used up to the present time the water repellent substance has consisted of a relatively long chain saturated aliphatic compound having 16 to 30 carbon atoms in the aliphatic chain, such as stearic acid, oleic acid, montanic acid, or the like, chemically combined with a coupling radical in the native quaternary ammonium compound, such as pyridinium chloride. An example of such a compound which is widely used in the production of water repellent cotton cloth is stearamido-methylpyridinium chloride. When applied in solution to a textile fiber or fabric to be rendered water repellent, and heated, the quaternary ammonium compound breaks down, causing a reaction with the cellulose of the fiber and affixing the long chain fatty radical more or less permanently to the textile fibers by a chemical linkage which has been variously termed an ether and an acetal linkage and imparting a degree of durable water repellency thereto.

These prior art water repellent compositions are not entirely satisfactory as most of them lose a great percentage of their water repellency ratings after four or five washings or even a lesser number of dry cleanings. They are also difficult to control and apply and unpleasant to work with. The destruction of the quaternary ammonium radical under the heat used to affix the water repellent composition to the fabric produces degradation products which must be removed from the fabric by further washings. The odor of pyridine coming from the drying ovens and wash tanks is unpleasant and irritating and often remains on the fabric after it enters the normal channels of commerce, where it causes further irritation to workers and users of such water repellent fabrics. Moreover, they are not useful to impart water repellency to non-cellulose fibers such as nylon, Orlon, wool, etc.

It is one of the objects of my invention to produce a durable water repellent composition which does not depend upon the use of a quaternary ammonium coupling radical to affix a water repellent residue to a textile fiber and avoids the disadvantageous features arising from the use of a compound containing that radical.

Another object of my invention is to provide a durable water repellent composition and method of application which does not produce degradation products which must be removed from the cloth and which produces a substantially odor-free water repellent fabric and process.

Another object of my invention is to provide water repellent textile fibers and fabrics which will at the same time have desirable spot resistance, crease proofing and lowered static electrical properties.

Another object of my invention is to provide water repellent compositions and methods of application of such compositions to textile fibers and fabrics which are equally applicable to a wide range of textile fibers and fabrics, such as cotton, artificial silk and other synthetic fibers.

Another object of my invention is to provide aqueous emulsions of water repellent materials containing long

2

chain fatty radicals which are stable under normal conditions of shipment and storage and which may be affixed to textile fibers and fabrics by ordinary resin curing steps, to impart more durable water repellent characteristics to textiles than the water repellents now in use.

Various other objects and advantages of my invention will appear as this description proceeds.

The effectiveness of methylene distearamide as a water repellent on cotton cloth has hereto been experimentally tested. In that work the methylene distearamide was applied to the cotton fabric as a solution in glacial acetic acid. That work showed that, unlike stearamido-methylpyridinium chloride, the compound showed no tendency to chemically bond itself to the cellulose, and the water repellent finish produced by the deposited compound was insufficiently resistant to laundering to be of practical value.

A glacial acetic acid solution of the methylene distearamide was used in this experimental work for the application of the compound to the cotton fabric because the compound was found difficult, if not impossible, to suspend as a colloid in an aqueous medium. I have invented a method by which I can secure a true colloidal dispersion of methylene distearamide and analogous compounds of relatively high molecular weight in an efficient and expeditious manner, which I have described and claimed in my copending application Serial No. 690,624, filed October 17, 1957, now U.S. Patent No. 2,972,548. That invention solved one of the major problems involved in the use of this class of compounds in rendering fibers and textiles water repellent. By that invention an aqueous stable colloidal dispersion consisting of a continuous phase comprising a solution of about 1 part to about 5 parts per 100 parts by weight of said colloidal dispersion of an acid-stable non-ionic surface active agent in water and a discontinuous phase comprising colloidal particles of a compound produced in situ having the formula  $(RCONH)_2CH_2$  in which R represents an aliphatic hydrocarbon chain containing 16 to 30 carbon atoms is obtained. By the present invention I provide a method for affixing the long-chain methylene diamines to fibers and textile fabrics so as to impart water repellency which is retained through several washings or dry cleaning operations, and thereby provide an improved water repellent finish which is superior to those now commercially available.

In accordance with this invention, I prepare an aqueous colloidal dispersion which has at least two dispersed phases and a continuous aqueous phase which has at least one surface active agent dissolved therein. One of these dispersed phases consists of colloidally dispersed particles of a compound having the generic formula



in which R represents an aliphatic hydrocarbon chain of 16 to 30 carbon atoms, such as, for example, methylene distearamide (or methylene diotadecyl amide), methylene dioleyl amide, methylene dimontan amide, etc.

The second dispersed phase of this complex colloidal dispersion consists of colloidally dispersed particles or droplets of a urea-formaldehyde resin, a modified urea-formaldehyde resin, a melamine-formaldehyde, a modified melamine formaldehyde or other resin which is heat-curing and dispersible as a colloidal suspension or dispersion. The resin utilized should be of a composition such that, after it is cured, it contains no free or unreacted soluble or deliquescent material, such as free urea, glycol, glycerol or the like.

A modified urea-formaldehyde resin which I have found suitable for use in this composition is a reaction product of urea, formaldehyde and methanol which is in substantially the monomeric stage. A resin of this type is sold

under the tradename of "Rhonite R-2." Another suitable resin is a methylated methylol melamine, such as "Aerotex M-3" or "Resloom M-75." Acetylene diureine formaldehyde resin is another suitable resin for my purpose.

When necessary to secure an expeditious cure of the particular heat-curing resin which forms the second dispersed phase of this complex dispersion, I include in the composition a catalyst which is adapted to hasten the curing of the particular resin involved. The catalyst used may be dissolved in the continuous aqueous phase of the composition or be emulsified as a third dispersed phase, depending upon its solubility in water. Citric acid and ammonium sulfate are suitable catalysts for expediting the heat-curing of a methylated methylol melamine resin. Zinc nitrate is a suitable catalyst for acetylene diureine formaldehyde resin. The amine hydrochloride catalysts, such as, for example, the hydrochloride of 2-amino-2-methyl-1-propanol (catalyst "A-C") are suitable for use with a urea-formaldehyde paste and may be added to the composition in an amount within the range of about 0.25% to about 2.00% by weight, of the composition.

This complex colloidal dispersion may contain additional dispersed phases comprised of other water insoluble materials which are used in the treatment of textiles, such as, for example, paraffin wax, stearic acid and the like. I have found that the addition of a mineral oil to the composition is advantageous in that it appears both to aid in the emulsification of other ingredients and to suppress any tendency of the composition to foam during its application to a textile fiber or fabric.

I have also found that this complex colloidal dispersion may advantageously contain a film-forming polymer emulsion that imparts no rewetting action and that is fully compatible with the other components of the emulsion. Such a film-forming polymer appears to reduce the tendency of the resin fixed methylene diamides to flake or dust off the fabric with use. Typical of such film-forming polymer emulsions that are compatible with the complex colloidal dispersion are polyvinyl acetate emulsion, polyacrylate emulsion, polystyrene emulsion and some synthetic rubber emulsions and latices.

In the preparation of this complex aqueous dispersion, I prepare a colloidal dispersion of a compound having the formula  $(RCONH)_2CH_2$  in which R represents an aliphatic hydrocarbon chain of 16 to 30 carbon atoms in an aqueous solution of a surface active agent. I may prepare this aqueous colloidal dispersion by the method described by my copending application Serial No. 690,624 referred to hereinbefore, although this invention is not limited to the preparation of the dispersion by that particular method or to the use of the particular colloidal dispersion claimed by that application.

The resin which forms the second dispersed phase of this complex aqueous dispersion may be dispersed directly in the aqueous dispersion of the  $(RCONH)_2CH_2$  compound. However, I prefer from a practical operating standpoint to prepare a second colloidal dispersion which carries the heat-curing resin as at least one of its dispersed phases and has a continuous phase comprising an aqueous solution of at least one surface active agent, and then mix this dispersion with the aqueous dispersion of the  $(RCONH)_2CH_2$  compound.

This second aqueous dispersion, carrying a heat-curing resin as a dispersed phase, may carry one or more textile treating materials, such as, stearic acid, paraffin wax, mineral oil, etc. as additional dispersed phases. This second dispersion may also carry the film-forming polymer emulsion as an additional dispersed phase. Alternatively, when it is desired to include such added textile treating materials in the final complex aqueous dispersion, they may be dispersed as discontinuous phases in one or more separate aqueous dispersions, and then these dispersions are mixed with the aqueous dispersion of the  $(RCONH)_2CH_2$  compound and of the heat-curing resin.

The first step of the method in accordance with this in-

vention for rendering a textile fiber or fabric water repellent consists of wetting the fiber or fabric with a complex aqueous colloidal dispersion comprising a dispersed phase consisting of particles of a compound having the generic formula  $(RCONH)_2CH_2$  in which the R represents an aliphatic hydrocarbon chain of 16 to 30 carbon atoms, a second dispersed phase consisting of particles or droplets of a heat-curing resin, such as, for example, a urea-formaldehyde resin, a modified urea-formaldehyde resin, a melamine-formaldehyde resin, a modified melamine-formaldehyde resin, mixtures of these resins, and the like with or without additional textile treating materials and a continuous phase comprising an aqueous solution of at least one surface active agent.

The wet fiber or fabric is then dried. It may be permitted to dry at normal atmospheric temperature, but is preferably dried at an elevated temperature to speed up the operation. The elevated temperature used to dry the fiber or fabric may be, for example, a temperature within the range of about 212° F. to about 250° F. After the fiber or fabric is dried, it is subjected to an elevated temperature adapted to cure the particular heat-curing resin involved for a period of which will effect its complete cure. Thus, the curing temperature may be within the range of about 290° F. to about 330° F. for a period of time within the range of about 5 to about 10 minutes. After this curing operation, the fiber or fabric is permitted to cool to room temperature.

The method in accordance with this invention is applicable to a wide range of textile fibers and fabrics, including cotton, viscose, cellulose acetate, and others. The treated fiber and fabric, in accordance with this invention, comprises individual fibers which carry a partial or complete coating of a compound of the generic formula  $(RCONH)_2CH_2$  in which R represents an aliphatic hydrocarbon chain of 16 to 30 carbon atoms which is bound to the fiber by a heat-cured synthetic resin. Treatment, in accordance with this invention, does not close the interstices of a fabric.

When the treatment includes a film-forming polymer emulsion it has been found that flaking or dusting of the resin from the fabric is better controlled and the treatment is more durable to both laundering and dry cleaning.

I have been unable to determine the exact mechanism by which the heat-cured resin bonds the  $(RCONH)_2CH_2$  compound to the fiber. However, the fact remains that the result is a durable, water repellent finish which is resistant to both laundering and dry cleaning. Thus, for example, a treated fabric, in accordance with this invention may have a spray rating of 100 and retain this rating through several launderings, or dry cleanings. Furthermore, the fibers and fabrics will, at the same time, have desirable spot resistance, crease-proofing and lowered static electrical properties.

The following examples illustrate practical applications of my invention, but it will be understood that the invention is not limited to the examples chosen for the purposes of illustration.

#### EXAMPLE I

##### *Methylene Distearamide Emulsion Preparation*

A mixture of the following ingredients were mixed together and refluxed for a period of one hour at a temperature of 96°-99° C.:

|                                        | Parts by weight |
|----------------------------------------|-----------------|
| Octadecylamide                         | 14.5            |
| Formaldehyde, 37% aqueous solution     | 5.8             |
| Sorbitan monopalmitate                 | 0.5             |
| Polyoxyethylene sorbitan monopalmitate | 0.5             |
| Water                                  | 60.0            |

justed to a value within the range of about 1 to about 4, preferably between 2.0 to 3.0 by the addition of about 0.9 part of hydrochloric acid. The mixture was then heated at 80° C. for an additional period of one hour and cooled to 60° C. Monoethanol amine was then added to neutralize the hydrochloric acid present. This required about 1 part of amine. An aqueous solution having the following composition was then added to the reaction mixture:

|                                        | Parts by weight |
|----------------------------------------|-----------------|
| Sorbitan monopalmitate                 | 1.5             |
| Polyoxyethylene sorbitan monopalmitate | 1.5             |
| Water                                  | 14.7            |

17.7

This mixture was then vigorously stirred and homogenized to produce a uniform, stable dispersion in which methylene distearamide is the dispersed phase and an aqueous solution of sorbitan monopalmitate and polyoxyethylene sorbitan monopalmitate is the continuous phase.

#### *Methylene Distearamide-Resin Emulsion*

The following ingredients were added to 15 parts by weight of the above-prepared methylene distearamide emulsion:

|                                                       |  |
|-------------------------------------------------------|--|
| 5 parts of modified urea-formaldehyde resin           |  |
| 1 part of monethanolamine hydrochloride as a catalyst |  |

and thoroughly admixed therewith. The resultant composition was then ready for use in the treatment of a textile fabric. The modified urea-formaldehyde resin used in this example consisted of a monomeric reaction product of urea, formaldehyde and methanol (Rhonite R-2).

#### *Fabric Treatment With Resin Emulsion*

Cotton corduroy was passed through a bath containing the above-prepared methylene distearamide-resin emulsion and thoroughly wet by the emulsion. The impregnated fabric was then dried and the resinous components carried thereon were cured at a temperature of 300° F. for 6 minutes.

The cotton corduroy treated in this manner for water repellency had an initial spray rating of 100. This rating remained unchanged through several launderings.

#### **EXAMPLE II**

##### *Methylene Distearamide Emulsion Preparation*

A mixture of the following ingredients were refluxed for 3/4 of an hour at a temperature of 195° F.-200° F.:

|                             | Parts by weight |
|-----------------------------|-----------------|
| Octadecylamide              | 20              |
| Formaldehyde (37% solution) | 8               |
| Sorbitan monopalmitate      | 1               |
| Water                       | 55              |

After this period of reflux, 4.6 parts by weight of dipropylene glycol was added to the reaction mixture and its pH was adjusted to a value within the range of about 1 to about 4, preferably between 2.0 and 3.0 by the addition of approximately 0.5 part by weight of 20° Baumé hydrochloric acid. The dipropylene glycol is added to keep the emulsion smooth; it also has foam suppressant properties. The resulting reaction mixture was then heated at 184°-188° F. for a period of one hour. The reaction mixture was then neutralized by the addition of approximately 0.4 part by weight of monoethanolamine, and then cooled, while stirring, to a temperature of 150° F.

#### *Methylene Distearamide-Resin Emulsion*

The following ingredients were then added to the resulting aqueous dispersion of methylene distearamide in

an aqueous solution of sorbitan monopalmitate and dipropylene glycol:

|                                  | Parts by weight |
|----------------------------------|-----------------|
| Modified urea formaldehyde resin | 5.0             |
| Mineral oil                      | 2.0             |
| Sorbitan monopalmitate           | 3.5             |

The additional emulsifier is added at this point to insure stability and freedom from flocculation. The resulting mixture was then stirred and permitted to cool until its temperature dropped to 100°-105° F., and was then passed through a colloid mill. The resin emulsion is then ready for use in treatment of fabrics as was done in Example I.

10 The following optional treatment can be made to the above prepared resin emulsion to improve the wash fastness of the finished water repellent treatment. This optional modification is best used for synthetic fibers and cloth containing synthetics; it may be omitted on cotton fabric and fibers as shown in Example I.

#### *Optional Melamine Resin Treatment*

The following ingredients were then added to 8 parts by weight of the above resulting colloidal suspension:

|                                    | Parts by weight |
|------------------------------------|-----------------|
| Methylated methylol melamine resin | 4               |
| Citric acid                        | 0.1             |

and thoroughly admixed therewith. The resulting composition was then ready for use in the treatment of a textile fiber or fabric.

#### *Fabric Treatment With Resin Emulsion*

35 Cotton corduroy was passed through a bath of the composition prepared as described above, and thoroughly wet by the composition. The impregnated fabric was then dried and the resinous components carried thereby cured at a temperature of 320° F. for a period of 7 minutes.

40 The cotton corduroy treated in this manner was tested for water repellency and for the durability of the water repellent finish deposited thereon by this treatment. The treated fabric was found to have an initial spray rating of 100. This rating remained unchanged through three successive dry cleanings, and still retained a spray rating of 80 after five successive washings, each conducted as prescribed by the No. 3 wash test of the American Association of Textile Chemists and Colorists.

#### **EXAMPLE III**

##### *Wax Emulsion Preparation*

A wax emulsion having the following composition was prepared:

|                                        | Parts by weight |
|----------------------------------------|-----------------|
| 55 Paraffin wax, 138° A.M.P.           | 20              |
| Stearic acid                           | 2               |
| Sorbitan monopalmitate                 | 3               |
| Polyoxyethylene sorbitan monopalmitate | 3               |
| Mineral oil                            | 2               |

60 The above mixture was heated to 225° F., whereupon it became clear. A mixture of four parts, by weight, of dipropylene glycol and 48 parts, by weight, of water, was heated to a temperature of 150° F. and added slowly to the foregoing mixture with good agitation. Eighteen parts of zirconyl acetate (13% ZnO<sub>2</sub>) were then added to the composition and uniformly admixed therewith. In place of zirconyl acetate, there can be used the equivalent amount of aluminum acetate (6% as 100% powder).

65 70 The composition was then passed through a colloid mill.

#### *Wax-Resin Emulsion*

Fifty parts by weight of this wax emulsion as prepared above was then admixed with fifty parts by weight, of the 75 methylene distearamide resin emulsion of Example II.

*Fabric Treatment With Resin Emulsion*

A textile treating bath was prepared from the foregoing wax-resin emulsion by adding the following ingredients to eight parts by weight of that composition:

|                               | Parts by weight |
|-------------------------------|-----------------|
| Urea-formaldehyde resin paste | 20              |
| Urea-formaldehyde polymer     | 3               |
| Amine hydrochloride catalyst  | 1               |

These ingredients were uniformly admixed into the composition, and the bath was ready for use. The urea-formaldehyde polymer utilized in this example was a high molecular weight reaction product of urea and formaldehyde ("Rhonite 414").

*Fabric Treatment With Resin Emulsion*

A viscose-acetate gabardine was passed through a bath of the composition described above and thoroughly wet by the composition. The gabardine was then dried and the resin which it picked up was cured by heating the fabric at a temperature of 320° F. for a period of six to seven minutes.

The gabardine treated in this manner was then tested for water repellency and for the durability of the water repellent finish deposited therein by this treatment. The treated fabric was found to have an initial spray rating of 100 and the water repellent finish was found to have excellent resistance to dry cleaning.

## EXAMPLE IV

*Methylene Distearamide Emulsion Preparation*

A mixture of the following ingredients were refluxed for 3/4 of an hour at a temperature of 195° F. to 200° F.

|                             | Parts by weight |
|-----------------------------|-----------------|
| Octadecylamide              | 22              |
| Formaldehyde (37% solution) | 9               |
| Sorbitan monopalmitate      | 1               |
| Water                       | 52              |

After this period of reflux, 5 parts by weight of di-propylene glycol was added to the reaction mixture and its pH was adjusted to a value within the range of about 1 to about 4, preferably between 2.0 and 3.0 by the addition of 20° Baumé hydrochloric acid. The resulting reaction mixture was then heated at 184°-188° F. for a period of one hour. The reaction mixture was then neutralized by the addition of monoethanolamine, and then cooled, while stirring, to a temperature of 150° F. An aqueous solution having the following composition was then added to the reaction mixture:

|                        | Parts by weight |
|------------------------|-----------------|
| Sorbitan monopalmitate | 3.5             |
| Mineral oil            | 2.0             |
| Water                  | 5.5             |

This mixture was then passed through a colloid mill.

*Methylene Distearamide-Additive Emulsion*

In order to provide a product that would not dust off or flake off after application to the fabric, to 90 parts by weight of the above emulsion were added:

|                                           | Parts by weight |
|-------------------------------------------|-----------------|
| Wax emulsion (as prepared in Example III) | 5               |
| Polyvinylacetate emulsion                 | 5               |

This composition was stirred until uniform.

*Methylene Distearamide-Resin Emulsion*

The following ingredients were added to 10 parts by weight of the above methylene distearamide-wax-polyvinyl-acetate emulsion:

|                               | Parts by weight |
|-------------------------------|-----------------|
| Urea-formaldehyde resin paste | 25              |
| Urea-formaldehyde polymer     | 3               |
| Amine hydrochloride catalyst  | 1               |

and thoroughly admixed therewith. The resultant composition was then ready for use in the treatment of a textile fabric. The urea-formaldehyde resin paste is a commercial preparation containing about 50% resin and about 50% water, and is sold as "Aerotex Cream 450."

*Fabric Treatment With Resin Emulsion*

A cotton fabric was passed through a bath containing the above prepared methylene distearamide-resin emulsion and thoroughly wet by the emulsion. The impregnated fabric was then dried and the resinous components carried thereon were cured as in the preceding examples.

The cotton fabric treated in this manner for water repellency had an initial spray rating of 100. The water repellent resin finish showed no dusting when flexed or subjected to a button-breaking operation.

It will be appreciated from the foregoing examples that the complex colloidal dispersions in accordance with this invention can be readily applied to textile fibers and fabrics and cured thereon to impart a durable water repellency which is more resistant to laundering and dry cleaning than the water repellents based on the use of long chain fatty radicals coupled with quaternary ammonium compounds, such as, stearamidomethylpyridinium chloride, which is widely used as the active ingredient in textile treating compositions of this type.

The heat-curing resin contained in these compositions, as already noted, bond the water repellent material, i.e., the  $(RCONH_2)_2CH_2$  compound, to the fibers to impart a durable water repellency to the fiber or fabric. In addition the cured resin imparts a crease-resistance to fabric which is an added advantage.

In carrying out the method of this invention there is no decomposition reaction which releases objectionable odors or leaves residues on the fiber. This is an important improvement over the compositions which utilize as an active ingredient a compound which contains a quaternary ammonium group. The widely used stearamidomethylpyridinium chloride decomposes with the release of objectionable odors and tends to leave an objectionable odoriferous residue on a textile fiber or fabric which are entirely avoided by my composition.

In the process of making the methylene distearamide emulsion, while I do not want to be bound by any theories regarding the reactions taking place, it is my belief that the chemical reaction involved here takes place in two steps. In the first step formaldehyde is believed to react with the long chain aliphatic amide to form a methyol derivative according to the following equation.



In the second step, this methyol derivative is believed to react, when under acid conditions, with an additional quantity of aliphatic amide to form the diamide, according to the following equation:



Thus, according to these theories, the product of the reaction of octadecyl amide (stearyl amide) with formaldehyde results in a product which has the following structural formula:



This compound is alternatively known as methylene distearamide or as distearamide methane.

While I have specifically exemplified the compositions, the method for their application and the water repellent fibers and fabrics, in accordance with my invention, it will be understood that these are for illustrative purposes

only and that various modifications and changes may be made in the various formulas and in the method for their preparation and application, without departing from the spirit of my invention or the scope of the following claims:

I claim:

1. A substantially organic solvent-free aqueous colloidal dispersion having a continuous phase comprising a solution of an acid-stable, non-ionic surface active agent selected from the group consisting of polyoxyethylene sorbitan monopalmitate and sorbitan monopalmitate in water, a discontinuous phase comprising colloidal particles of a compound produced in situ having the formula  $(RCONH)_2CH_2$  in which R represents an aliphatic hydrocarbon chain containing 16 to 30 carbon atoms and a second discontinuous phase comprising a heat-curable compound selected from the group consisting of methylol urea, methanol modified methylol urea, methylol melamine, and methylated methylol melamine.

2. A substantially organic solvent-free aqueous colloidal dispersion having a continuous phase comprising a solution of an acid-stable, non-ionic surface active agent selected from the group consisting of polyoxyethylene sorbitan monopalmitate and sorbitan monopalmitate in water, a discontinuous phase comprising colloidal particles of a compound produced in situ having the formula  $(RCONH)_2CH_2$  in which R represents an aliphatic hydrocarbon chain containing 16 to 30 carbon atoms and a second discontinuous phase comprising a heat-curable compound selected from the group consisting of methylol urea, methanol modified methylol urea, methylol melamine, and methylated methylol melamine, and a third discontinuous phase comprising a film-forming polymer selected from the group consisting of polyvinylacetate and polystyrene.

3. A substantially organic solvent-free aqueous colloidal dispersion having a continuous phase comprising a solution of an acid-stable, non-ionic surface active agent selected from the group consisting of polyoxyethylene sorbitan monopalmitate and sorbitan monopalmitate in water, a discontinuous phase comprising colloidal particles of a compound produced in situ having the formula  $(RCONH)_2CH_2$  in which R represents an aliphatic hydrocarbon chain containing 16 to 30 carbon atoms, a second discontinuous phase comprising a heat-curable compound selected from the group consisting of methylol urea, methanol modified methylol urea, methylol melamine and methylated methylol melamine, a third discontinuous phase comprising mineral oil, and a catalyst adapted to hasten the curing of the heat-curable compound.

4. A substantially organic solvent-free aqueous colloidal dispersion having a continuous phase comprising a solution of an acid-stable, non-ionic surface active agent selected from the group consisting of polyoxyethylene sorbitan monopalmitate and sorbitan monopalmitate in water, a discontinuous phase comprising colloidal particles of a compound produced in situ having the formula  $(RCONH)_2CH_2$  in which R represents an aliphatic hydrocarbon chain containing 16 to 30 carbon atoms, a second discontinuous phase comprising heat-curable methanol modified methylol urea, and a catalyst adapted to hasten the curing of said methylol urea.

5. A substantially organic solvent-free aqueous colloidal dispersion having a continuous phase comprising a solution of an acid-stable, non-ionic surface active agent selected from the group consisting of polyoxyethylene sorbitan monopalmitate and sorbitan monopalmitate in water, a discontinuous phase comprising colloidal particles of a compound produced in situ having the formula  $(RCONH)_2CH_2$  in which R represents an aliphatic hydrocarbon chain containing 16 to 30 carbon atoms, a second discontinuous phase comprising heat-curable

methylol urea and a catalyst adapted to hasten the curing of the said methylol urea and a third discontinuous phase comprising film-forming polyvinylacetate.

6. A substantially organic solvent-free aqueous colloidal dispersion having a continuous phase comprising a solution of an acid-stable, non-ionic surface active agent selected from the group consisting of polyoxyethylene sorbitan monopalmitate and sorbitan monopalmitate in water, a discontinuous phase comprising colloidal particles of a compound produced in situ having the formula  $(RCONH)_2CH_2$  in which R represents an aliphatic hydrocarbon chain containing 16 to 30 carbon atoms, a second discontinuous phase comprising heat-curable methylated methylol melamine and a catalyst adapted to hasten the curing of the said methylol melamine.

7. A substantially aqueous colloidal dispersion consisting of a continuous phase of a solution of an acid-stable, non-ionic surface active agent selected from the group consisting of polyoxyethylene sorbitan monopalmitate and sorbitan monopalmitate in water, a discontinuous phase consisting of colloidal particles of methylene distearamide produced in situ, a second discontinuous phase consisting of a heat-curable compound selected from the group consisting of methylol urea, methanol modified methylol urea, methylol melamine, and methylated methylol melamine, and a catalyst adapted to hasten the curing of the said heat-curable compound, and a third discontinuous phase consisting of a film-forming polymer selected from the group consisting of polyvinyl acetate and polystyrene.

8. A substantially aqueous colloidal dispersion consisting of a continuous phase of a solution of polyoxyethylene sorbitan monopalmitate and sorbitan monopalmitate in water, a discontinuous phase consisting of colloidal particles of methylene distearamide produced in situ, a second discontinuous phase consisting of heat-curable methanol modified methylol urea, and a catalyst adapted to hasten the curing of the said methylol urea.

9. A substantially aqueous colloidal dispersion consisting of a continuous phase of a solution of sorbitan monopalmitate in water, a discontinuous phase consisting of colloidal particles of methylene distearamide produced in situ, a second discontinuous phase consisting of heat-curable methylol urea, and a catalyst adapted to hasten the curing of the said methylol urea, and a third discontinuous phase consisting of film-forming polyvinyl acetate.

10. A substantially aqueous colloidal dispersion consisting of a continuous phase of a solution of an acid-stable nonionic surface active agent selected from the group consisting of polyoxyethylene sorbitan monopalmitate and sorbitan monopalmitate in water, a discontinuous phase consisting of colloidal particles of methylene distearamide produced in situ, a second discontinuous phase consisting of heat-curable methylated methylol melamine, and a catalyst adapted to hasten the curing of said methylol melamine.

#### 60 References Cited in the file of this patent

#### UNITED STATES PATENTS

|           |                 |               |
|-----------|-----------------|---------------|
| 2,423,428 | Pollard         | July 1, 1947  |
| 2,491,249 | Cathers et al.  | Dec. 13, 1949 |
| 2,505,649 | Pikl            | Apr. 25, 1950 |
| 2,511,113 | La Piana et al. | June 13, 1950 |
| 2,861,054 | Rust et al.     | Nov. 18, 1958 |
| 2,981,704 | Herbes et al.   | Apr. 25, 1961 |

#### OTHER REFERENCES

Schwartz et al.: "Surface Active Agents and Detergents," volume II (1958), Interscience Pub. Inc., New York, page 134.